

June 24, 1924.

1,498,908

C. G. FINK

EVACUATED CONTAINER

Filed Jan. 23, 1915

Fig. 1.



Fig. 2.



Witnesses:

E. Tujakowski

J. Ellis Glen.

Inventor:

Colin G. Fink,

by *Alfred H. Davis*  
His Attorney.

Patented June 24, 1924.

1,498,908

# UNITED STATES PATENT OFFICE.

COLIN G. FINK, OF EAST ORANGE, NEW JERSEY, ASSIGNOR TO GENERAL ELECTRIC COMPANY, A CORPORATION OF NEW YORK.

## EVACUATED CONTAINER.

Application filed January 23, 1915. Serial No. 4,048.

To all whom it may concern:

Be it known that I, COLIN G. FINK, a citizen of the United States, residing at East Orange, county of Essex, State of New Jersey, have invented certain new and useful Improvements in Evacuated Containers, of which the following is a specification.

This application is in part a continuation of my prior application, Serial No. 703,801, filed June 15, 1912.

My invention relates to seals for leading-in conductors for incandescent lamps, gas electric lamps, mercury rectifiers and apparatus of a similar nature in which an envelope of glass or vitreous material is used and in which it is necessary to provide means for conducting electrical energy from a power circuit to conductors within the space enclosed by the envelope.

In order to make a seal for such apparatus which will be gas-tight, the leading-in conductor used should preferably have a coefficient of expansion which does not differ greatly from that of the material of the envelope. It is also necessary that there shall be a certain affinity between the material of the envelope, when in a plastic or partially liquid condition, and the surface of the conductor, by reason of which there will be a tendency for the two to stick together. This property is usually spoken of as a "wetting" of the conductor by the material of the envelope. When the envelope consists of ordinary glass, platinum has been found especially suitable for a leading-in conductor because of the fact that it is practically non-oxidizable and has a coefficient of expansion which is nearer to that of the glass than any other metal, and also because platinum is "wet" by glass. Because of the great cost of platinum, however, many efforts have been made to secure a suitable substitute. It has been found that if nickel and iron are alloyed in the proper proportions, a conductor may be obtained which has the same coefficient of expansion as glass. In attempting to use such a conductor in commercial practice, however, difficulty has been experienced because of the large number of seals which are defective. This is probably due to the fact that when subjected to the heat of the flame necessary for the sealing-in operation an oxide coating is formed which is more or less porous and allows air to gradually leak through between

the glass and the conductor. It has also been found difficult to prevent the formation of bubbles in the seal due to the liberation of gas from the conductor or the formation of gas by chemical reaction during the sealing-in operation.

I have discovered, however, that there are certain metals whose oxides are readily soluble in glass at lamp seal making temperatures. Among these are copper and cobalt and some of their alloys. Ordinary lead glass, such as is commonly used for incandescent lamps and rectifiers, has a coefficient of expansion of about  $8.8 \times 10^{-6}$  while copper and cobalt have coefficients of expansion of about  $17 \times 10^{-6}$  and  $12 \times 10^{-6}$  respectively. Hence, solid conductors composed entirely of either of these metals are not commercially suitable for leading-in conductors because of the great difference between their coefficients of expansion and that of glass. By making a composite conductor, however, having a sheath of copper or cobalt and a core of metal having a lower coefficient of expansion than that of glass, and by properly proportioning the relative thicknesses of the core and sheath, it is possible to provide a conductor, the total radial coefficient of expansion of which is substantially the same as that of the glass with which it is to be used. I have found that if such a conductor is used that there is an even better union in the cold state between the conductor and the glass than in the case of platinum. In actual practice it has been found that by using my invention the number of defective seals has been reduced over 75% from the number commonly found when platinum is employed.

Most metals have a coefficient of expansion greater than that of glass and hence cannot be used to form a core for the composite conductor. Among those metals having a sufficiently low coefficient are tungsten and molybdenum, which have coefficients of about  $4.3 \times 10^{-6}$  and  $4.9 \times 10^{-6}$  respectively. There are, in addition to these metals, various alloys which can be readily prepared which have a coefficient of expansion less than that of lead glass. For example, an alloy of nickel and iron containing about 35% of nickel has a coefficient of expansion which is practically zero over a range of temperature from  $0^{\circ}$  to  $100^{\circ}$  C. By vary-

ing the relative amounts of nickel and iron, it is possible to produce an alloy having any coefficient desired between zero and that of nickel or iron. One alloy which I have used with satisfactory results contains from 53 to 55% of iron, from 44 to 46% of nickel, and from .75 to 1.25% of manganese, and not over .15% of carbon, .02% of phosphorus, .20% of silicon and .02% of sulphur. 10 The presence of a small amount of manganese ensures an easy drawing metal and I believe that it also assists in counteracting the tendency on the part of the finished wire to form bubbles when being sealed into glass, 15 while the presence of some of the impurities apparently causes the formation of bubbles.

The coefficient of expansion of the core material will vary considerably with different lots of metal due to small variations in the proportions of the constituents and on this account it will be necessary in each case to measure the coefficient of expansion of the core and sheath and the diameter of 25 the core and from the values found calculate the required thickness of sheath to give a finished conductor having substantially the same coefficient as the glass with which it is to be used. The lamp glass commonly 30 used has a coefficient of expansion slightly below that of platinum. One example of a composite wire suitable for such glass has a core of the above described nickel iron alloy containing about 44% nickel and a 35 copper sheath of which the thickness expressed in per cent of the diameter of the core is approximately 6%, the approximate percentage of copper being about 20% by volume of the total volume of the wire.

40 There are numerous ways in which the copper sheath may be applied to the core. I prefer, however, to employ what I term the copper tube process. The alloy having the desired proportions for the core is made 45 up into rods. These rods as received from the rolling mill are usually rough and not perfectly round, and may be polished or drawn through dies to give them a smooth 50 clean surface. They should then be thoroughly heat-treated at a temperature of about 1200° to 1300° C. in an atmosphere of hydrogen or hydrogen diluted with nitrogen. The time of this heat treatment will 55 depend somewhat upon the diameter of the rods. I have found that when the rods of the particular alloy which I have mentioned are about one-half inch in diameter from 8 to 10 hours is necessary. After subjecting them to the temperature mentioned 60 for the desired period, I find it desirable to allow the rods to cool slowly in a hydrogen or hydrogen-nitrogen atmosphere. This prevents oxidation of the surface. In addition to rendering the metal more easily workable, this heat treatment also prevents

the formation of bubbles in the glass when a seal is made. This is probably due to the fact that the hydrogen acting upon the heated alloy removes impurities such as carbon and possibly sulphur. I have found that if the heat treatment is continued until the rods contain no more than .02% of carbon, the tendency of the sheathed wire to form bubbles is eliminated.

70 It is essential that there should be a perfect union between the core and the sheath as otherwise the conductor will not draw well and there will be danger of air leaking between the core and sheath after the seal has been made. In order to ensure a perfect joint between the sheath and the core, the latter may be given a very thin coating 75 of copper, by dipping for a short time in a bath of copper sulphate, and then a coating of silver or brass. Before applying the second coating the rods may be heated to the melting point of copper causing the thin film of copper to alloy with the core metal. This insures a better sticking surface for the 80 second coating. This second coating, which may be plated on the rods or may be applied in the form of a thin sheet wound around the rods, should preferably have a melting point below that of copper. After 85 the rod has been heat-treated and coated in this way, a copper tube is selected having the required diameter and thickness. This tube is slipped over the core rod and made to fit tightly by drawing. The sleeved rods are then placed in a furnace and heated under non-oxidizing conditions, preferably in 90 hydrogen or hydrogen diluted with nitrogen, to a temperature slightly above the melting point of the silver or brass with 95 which the cores are coated. The heated rods are then run through rolls to insure a close union between the core and sheath. Upon cooling the core and sheath will be 100 found to be firmly soldered together. The rods thus prepared are then ready to be 105 drawn into wire according to the usual methods. In drawing down to the desired size I find that it is desirable at frequent intervals, as, for example, after each reduction of about 40 mils in diameter, to anneal the wire for one hour at a temperature 110 of about 900° C. in a non-oxidizing atmosphere, preferably hydrogen. When prepared in this way, the coefficient of expansion 115 of the finished annealed wire will be found to be substantially the same as the value calculated and the adherence between the sheath and core will be perfect.

120 Before using the composite wire thus obtained for making seals it may be found desirable to apply to it a coating of a borate. Borax is suitable for this purpose though zinc borate and other borates also may be used. Zinc borate is especially suitable because of the fact that it is non-hygroscopic 125 130

and no special precautions are necessary for preserving the wire from moisture between the time when it receives the coating and the time it is used. The desired coating may be applied by passing the wire through a solution or suspension of the borate and then heating to a temperature sufficient to drive off all water from the coating which adheres to the wire and to thoroughly harden the coating. This coating serves a double purpose; it serves to protect the wire during the sealing-in operation and also facilitates the solution or absorption of the oxide film by the glass. When a wire prepared in this way is sealed into glass under proper temperature conditions, a remarkably close adherence between the glass and the wire is obtained. Just why this is true it is difficult to state precisely. A microscopic examination of such a seal, however, reveals the fact that there is between the glass and the copper sheath some material of different composition which apparently binds the two together. This binding material may be composed principally of the oxide which covers the wire but, from the fact which has been proved by careful experiment that it is possible to dissolve all of the oxide coating in the glass, it seems more probable that a portion at least of the oxide is dissolved in the glass and that the glass is more or less mingled with the remaining portion of the oxide, thus producing a firm adherence between the glass and the oxide coating as well as filling the pores in the oxide. Whatever the composition of the binding material may be, it produces a more intimate union between the wire and the glass than in the case of a platinum seal. This may be shown by crushing both a seal made with platinum and a seal made with a composite wire prepared as I have described. The glass will break away cleanly from the platinum while small particles of the broken glass will be found adhering closely to the composite wire and particles of the coating of the wire will be found sticking to the glass that has been broken away. This would seem to indicate that the union between platinum and glass is somewhat of the nature of a good mechanical joint while a wire such as I have described will be so closely united to the glass that the two cannot be separated without tearing. The union between glass and platinum is not strong enough to prevent a plain piece of platinum wire from being drawn through the glass after it has been sealed in.

In the accompanying drawing which illustrates my invention, Fig. 1 represents an incandescent lamp having a seal made in accordance with my invention, and Fig. 2 is a cross section, greatly magnified, of a portion of the seal. As shown in the drawing the incandescent lamp 1 has the usual leading-in

conductors 2, 2, sealed through the stem 3. In making seals with platinum it has been customary, because of the high cost of this metal, to use only a short section of platinum wire where the leading-in conductor 70 passes through the glass of the stem and for the remaining portion of the conductor to use a wire of cheaper metal having good conductivity. In many cases it will be desirable to employ a similar construction 75 when the seal is made according to my invention. Because of the comparative cheapness of my wire, however, this will not be necessary from the standpoint of cost and if desired the entire leading-in conductor may, as indicated in the drawing, be made of the wire which I have described. In case this construction is employed it may be desirable to increase the mechanical strength of the seal by nicking or bending or crimping, as 85 indicated, that portion of the wire which passes through the glass of the stem.

When a section of a seal made in accordance with my invention is examined microscopically it will be found that the sheath 90 4 of the conductor, as illustrated in Fig. 2, is closely joined to the core 5 and that between the sheath and the glass body 6 there is a thin layer of binding material 7 which closely surrounds the conductor and which seems to merge into the glass.

If the coefficient of expansion of the wire is adjusted so that it is substantially the same as that of glass, the strains set up in the glass when the seal is made will be reduced to a minimum. If, however, the wire employed has a greater coefficient of expansion than ordinary glass, when the seal cools the wire tends to shrink away from the glass and the union between the two is under tension. On the other hand if the coefficient of expansion of the wire is materially less than that of glass the union between the glass and the wire when cooled will be under compression and there will be danger of the 105 glass around the wire cracking.

The sealing-in operation may be carried on with the apparatus ordinarily used for making seals with platinum wire. While it has usually been considered necessary heretofore, when attempts have been made to use an oxidizable wire, to carry on the sealing-in operation under non-oxidizing conditions I have found that such precautions are unnecessary with my composite wire and that the formation of oxide on the surface of the wire appears to be of distinct advantage instead of being detrimental. The sealing-in flames should of course be so adjusted that the temperature will be below the 115 melting point of the copper or other metal of which the sheath is composed. I have found that in some cases when the temperature used approaches too closely the melting point of the metal, all of the oxide on

the wire is apparently dissolved in the glass and that seals made under such conditions are often imperfect. This may be caused by a poor adherence between the glass and the bare copper of the sheath. On the other hand if the temperature employed is too low the seal may be imperfect owing to imperfect union between the wire and the glass. If the seal has been made at the proper temperature the wire in the finished seal will have a cerise or cherry red color while if the temperature is too low the wire will be dark red or black. These differences in the appearance of the seal permit an efficient inspection of the seals and the rejection of imperfect seals before they are placed in lamps, while with seals made with platinum or a platinum sheathed wire no difference is apparent between perfect and imperfect seals.

The conductivity of my composite wire may be made about two times that of pure platinum or three times that of commercial platinum and seven times that of nickel iron wire having the same coefficient of expansion. Hence it is possible to use much smaller wires for a given current carrying capacity and the smaller the wire used the easier it is to make perfect seals.

30 What I claim as new and desire to secure by Letters Patent of the United States, is,—

1. An article of manufacture comprising a vitreous body and a composite wire sealed therein, said wire having an outer sheath of cupreous metal with a thermal expansion higher than that of said vitreous body and a core of metallic material with a thermal expansion lower than that of said vitreous body, said sheath and core being united and so proportioned that the wire has a thermal expansion such as to secure a seal with said vitreous body.

2. An article of manufacture comprising a body of vitreous material, and a composite wire sealed therein, said wire being composed of a core of alloy containing nickel and iron, and a cupreous outer sheath of which the oxide is combined with said vitreous material to form a thin layer of binding material firmly adherent to both the wire and the vitreous material.

3. An article of manufacture comprising a vitreous body and a wire of substantially the same thermal expansion as said vitreous body hermetically sealed therein and surrounded by a thin composite layer containing material from said wire combined with said vitreous body and firmly adherent to both said wire and said vitreous body.

4. An article of manufacture comprising a body of glass, and a composite wire composed of a cupreous sheath, and a core having a thermal expansion less than that of said glass, said wire and sheath being proportioned to render the thermal expansion

of the wire substantially the same as that of the glass, said wire being hermetically sealed into said body of glass and having a cerise or cherry red color where it is surrounded by the glass.

5. A composite low expansion wire comprising a core of nickel steel and an external copper sheath welded thereto, said wire as a whole having less expansion than platinum.

6. A composite low expansion wire comprising a core of nickel steel and an external sheath of a metal of the copper class welded thereto, said wire as a whole having less expansion than platinum.

7. As a new article of manufacture, a copper surfaced wire having a rate of expansion as a whole below that of platinum.

8. As a new article of manufacture, a composite wire having a surface of base metal and having a rate of expansion as a whole below that of platinum.

9. As a new article of manufacture, a wire having a surface of metal of the copper class and a rate of expansion as a whole below that of platinum.

10. A 2-layer composite wire, one such layer being of low-expansion nickel steel and the other layer of high-expansion high-melting metal, the wire as a whole having an expansion less than that of platinum.

11. As a lamp wire, reinforced copper surface wire, said reinforcement consisting of an interior layer of low expansion nickel-iron alloy.

12. As a lamp wire, a composite wire composed of a layer of copper and another layer of low expansion nickel-steel in sufficient amount to reduce the total expansion sufficiently to secure a seal with lamp glass.

13. A leading-in wire comprising an outer sheath of high-melting, high-conductive material united to a core of nickel-steel having an average coefficient of expansion distinctly below that of the sheath, the core being under compression by the sheath at all temperatures to which the wire is subjected in lamp-making use.

14. The combination, with a gas-tight receptacle having a wall of vitreous material, of a composite leading-in wire sealed therein, said wire consisting of reinforced copper wire, said reinforcement consisting of a layer of low-expansion nickel-iron alloy.

15. The combination, with a gas-tight receptacle having a wall of vitreous material, of a composite leading-in wire sealed therein, said wire being composed of a layer of copper and another layer of low-expansion nickel-steel in sufficient amount to reduce the total expansion of the composite wire sufficiently to secure a seal with the glass.

16. The combination, with a gas-tight receptacle having a wall of vitreous material, of a composite leading-in wire sealed therein, said wire having a surface sheath of high-

melting base metal and a core of metallic material, the thermal expansion of the core and sheath being different and so proportioned as to produce a resultant expansion 5 of the composite wire such as to secure a seal with the glass.

17. The combination, with a gas-tight receptacle having a wall of vitreous material, of a composite leading-in wire sealed there-  
10 in, said wire having a surface sheath of copper and a core of metallic material, the ther-

mal expansion of the core and sheath being different and so proportioned as to produce a resultant expansion of the composite wire such as to secure a seal with the glass. 15

In witness whereof, I have hereunto set my hand this 21st day of January, 1915.

COLIN G. FINK.

Witnesses:

S. N. WHITEHEAD,  
J. H. ELKINS.